

June 6, 1944.

G. EHRENFRIED

2,350,736

METHOD OF PRODUCING DYE IMAGES

Filed July 10, 1942

FIG. 1.



FIG. 2.

INCOMPLETE  
BLEACHING



GEORGE EHRENFRIED  
INVENTOR

BY *Newton M. Penning*  
*R. Frank Smith*  
ATTORNEYS

## UNITED STATES PATENT OFFICE

2,350,736

## METHOD OF PRODUCING DYE IMAGES

George Ehrenfried, Rochester, N. Y., assignor to  
Eastman Kodak Company, Rochester, N. Y., a  
corporation of New Jersey

Application July 10, 1942, Serial No. 450,386

13 Claims. (Cl. 95—88)

This invention relates to a method for producing colored photographic images and particularly to a method of forming colored images in a dye-bleaching process of color photography.

Christensen, U. S. Patent 1,517,049, November 25, 1924, describes a process for producing a dye image in which a dyed gelatin layer containing a silver image is treated with a solution of a strong reducing agent such as sodium hydrosulfite or stannous chloride. The reducing bleach bath destroys the dye in the layers selectively in the region of the silver image, giving a positive dye image from a negative silver image. The destruction of a dye to form a photographic image in this process appears to depend upon the catalytic action of the silver image which results in the destruction of the dye in that portion of the film when treated with a suitable reducing bleach bath.

I have found that in some cases image-forming dyes used in this process may be more readily bleached if a freshly developed silver image is used rather than a silver image which has been washed or which has been treated with a fixing bath subsequent to reduction.

It is, therefore, an object of my invention to provide a novel method of forming a colored photographic image in a photographic layer. A further object is to provide a novel method for destroying a dye uniformly dispersed in a photographic layer under influence of a redeveloped silver image. Other objects will appear herein-after.

These objects are preferably accomplished, according to my invention, by exposing and developing the emulsion layer containing the uniform dispersion of image-forming dye, fixing, rehalogenizing the silver image thus formed, redeveloping the rehalogenized silver image, then treating the layer with a solution of a suitable reducing bleaching agent to bleach the dye from the layer in the region of the silver image.

Other objects are accomplished by repeating as many times as required the steps of rehalogenizing, redeveloping and bleaching in order that any dye remaining unbleached in the region of the silver image, may be bleached from the layer.

The photographic element treated according to my invention may comprise a single emulsion layer or a plurality of emulsion layers coated on one or both sides of a suitable support. This support may be a cellulosic material such as pigmented cellulosic material, synthetic resin or paper. The emulsion layer or layers may contain

5 a uniformly dispersed dye prior to exposure or a dye intermediate in which a colored compound may be formed after exposure. I prefer to use certain bleachable dyes of the general class of poly-azo dyes as disclosed in Christensen U. S. Patent 1,517,049, though not necessarily the same dyes, and bleachable azo dyes such as disclosed in my prior U. S. Patent 2,322,001, granted June 15, 1943. Certain bleachable vat dyes, as for instance those disclosed in Seymour U. S. Patent 2,184,022, granted December 19, 1939, are likewise suitable.

10 If a three-layer photographic element is used for the production of natural color images, the three emulsion layers preferably contain dyes, each of which is roughly complementary in color to the effective sensitivity of the emulsion layer. The red, green and blue sensitive emulsion layers may be colored roughly complementary to their sensitivity with azo dyes as shown in my prior application above-cited, or with vat dyes such as those shown in the above Seymour patent.

15 The layers need not be colored complementary to their sensitivity, however, but may be colored alternatively with a dye that transmits the colors for which the layers are mainly sensitive.

20 My invention is illustrated by Figs. 1 and 2 of the accompanying drawing. In the drawing, Fig. 1 shows in enlarged cross-sectional view the appearance of a color film in five stages of processing in accordance with the preferred manner of my invention. Fig. 2 shows in enlarged cross-sectional view the appearance of a color film which has been incompletely bleached in the processing steps illustrated in Fig. 1, which film is subjected to the processing steps shown in the last three stages of Fig. 1 in order to complete the bleaching of the dyes in the emulsion layers.

25 A film of the type shown in the first stage of Fig. 1 of the drawing or a single layer film, having emulsion layers or layer colored in relation to the sensitivity as described in my prior application, i. e. colored complementary to the sensitivity, is exposed in a camera or under a suitable color positive or negative. For example, it may be exposed to a natural color transparency by a single exposure to tungsten light through 30 suitable correcting filters or by three simultaneous or successive exposures to light transmitted by red, green and blue filters in a suitable ratio of times and intensities. The film is then developed in an ordinary black-and-white developer, washed and fixed. The silver image or

images is then reconverted to a silver halide such as silver chloride and the rehalogenized silver image or images are developed and the dyes bleached by treatment with a reducing bleach bath as for instance alkali stannite solution, neutral, or slightly acid or alkaline sodium hydro-sulfite, etc., with or without the addition of chemicals capable of accelerating bleaching. It is, according to my invention, the steps of redeveloping the rehalogenized silver image and using it for the bleaching of dye in an emulsion layer, which enhance the bleaching activity of the silver for dyes, particularly for dyes which are not readily bleached by the first developed silver image. Typical of such difficultly bleached dyes are Pontamine Fast Green 5BL and tetrazotized 4,4'-diamino-3,3',6,6'-tetramethyl tri-phenylmethane coupled with N-heptoyl H acid.

I have also found that in certain cases where the dyes are not completely bleached in the usual time of bleaching, in presence of the freshly developed silver image, it is advantageous to repeat the steps of rehalogenization, redevelopment and bleaching. These added processing steps appear to be necessitated, by certain of the dyes used, i. e. the difficulty with which certain dyes are bleached, and also by the character of the developed silver image. That is, a freshly developed silver image may have a much greater influence for bleaching dyes than an originally developed silver image which has been fixed and washed, so that the effective bleaching activity of the image may be enhanced by again producing it in the freshly developed state and using it to bleach more dye.

This part of my process wherein the steps of rehalogenization, redevelopment and bleaching are repeated, constitutes a cycle of steps which may be repeated as often as desired or as required by the particular color process in use.

In the process described in my prior application above-cited, wherein dyes are bleached under influence of a rehalogenized silver image, I also find that the steps of rehalogenizing and bleaching are advantageously repeated to obtain more effective or efficient bleaching of dyes in a photographic layer.

My invention will now be described by example and with particular reference to the figures of the accompanying drawing.

Fig. 1 shows a color film having emulsion layers colored in the manner described in my prior application, that is, the film has a support 10 of a cellulose ester or other suitable material carrying emulsion layers 11, 12, and 13 sensitized to red, green and blue light, and colored cyan, magenta and yellow, respectively. Layer 15 is a separating colloid layer containing a yellow filter material, as for example, colloidal silver, and layer 14 contains colorless colloidal material such as gelatin.

The film of Fig. 1 is exposed to a natural color transparency by a single exposure to tungsten light through suitable correcting filters. The film is then developed for about eight minutes at 68° F. in a tank of the following developer:

|                                  |       |     |
|----------------------------------|-------|-----|
| Monomethyl-p-aminophenol sulfate | grams | 2   |
| Hydroquinone                     | do    | 5   |
| Sodium sulfite (desiccated)      | do    | 100 |
| Borax (granular)                 | do    | 20  |
| Water to                         | liter | 1   |

The print is now placed for two minutes in a stop bath consisting of: acetic acid, 28 per cent, 500 cc.; water 4 liters.

The film is then thoroughly fixed in acid hypo solution of the following composition:

|                       |       |     |
|-----------------------|-------|-----|
| Water (about 125° F.) | cc    | 600 |
| Hypo                  | grams | 240 |
| Sodium sulfite        | do    | 15  |
| Acetic acid (28%)     | cc    | 48  |
| Boric acid crystals   | grams | 7.5 |
| Potassium alum        | do    | 15  |
| Water to              | liter | 1   |

The film now appears as shown in the second stage of Fig. 1 wherein the emulsion layers 11, 12, and 13 contain negative-silver in areas 21, 22, and 23, respectively in addition to dye.

15 The silver images produced by the development are bleached to silver chloride by treatment for about ten minutes in the following solution:

|                                 |       |     |
|---------------------------------|-------|-----|
| Cupric chloride                 | grams | 100 |
| Hydrochloric acid, concentrated | cc    | 25  |
| Water to                        | liter | 1   |

The film now appears as shown in the third stage of Fig. 1 wherein the emulsion layers 11, 12, and 13 contain the rehalogenized silver images 31, 32, and 33 respectively, and the emulsion layers are still uniformly colored throughout.

25 The film after exposure is then redeveloped in the above black-and-white developer and appears as shown in the fourth stage of Fig. 1 of the accompanying drawing, wherein the emulsion layers 11, 12, and 13 contain freshly developed silver images in areas 41, 42, and 43 respectively.

Without washing, the film is next placed in an alkaline stannous chloride solution which bleaches dyes selectively in the presence of the freshly developed silver images. The following sodium stannite solution is suitable for this purpose:

|                               |       |     |
|-------------------------------|-------|-----|
| Stannous chloride             | grams | 8   |
| 40 Water (distilled) to       | cc    | 100 |
| Sodium hydroxide 10% solution | do    | 100 |

The film is now washed in water. The silver images are then bleached in the same copper chloride bath previously used, to convert them to silver chloride, and thereafter, the silver chloride is removed from the emulsion layers by fixing in acid hypo bath of the same composition as that previously used.

55 50 The film appears as shown in the fifth stage of Fig. 1 wherein the layers 11, 12, and 13 have clear areas in the portions 51, 52 and 53 respectively. Layer 15 is clear, the filter material having been removed during the process of treatment with the cupric chloride and fixing solutions.

55 As mentioned above, I sometimes find that even by application of the novel method above described, the dyes may not be completely removed from the emulsion layers in areas from which it is intended that they should be removed to give a picture in natural colors. In Fig. 2, I have shown the appearance of a film of the type shown in the first stage of Fig. 1, which has been exposed, developed, fixed, rehalogenized, redeveloped, and bleached, and in which emulsion layer 13 is shown as having a completely bleached area 63, whereas areas 61 and 62 of layers 11 and 12 represent cyan and magenta dyes, respectively, which have not been removed during bleaching.

60 65 70 According to another feature of my invention I take this film shown in Fig. 2 of the accompanying drawing and repeat the steps of rehalogenizing, redeveloping and bleaching to obtain complete removal of dye in areas 61 and 62. 75 Thereafter, the silver images remaining in the

layers are converted to silver chloride by use of the same cupric chloride solution mentioned above and the resulting silver chloride images are removed with a hypo solution of the composition given above. The film then appears as shown in the fifth stage of Fig. 1 the areas corresponding to 51, 52, and 53 being clear.

In place of the copper chloride bleach bath used to convert the silver images to silver chloride, baths of the following composition may be used:

- A. Quinone, hydrochloric acid and ethyl alcohol.
- B. Ferric chloride and hydrochloric acid.
- C. Ammonium persulfate and hydrochloric acid.

In some cases it is desirable to add an organic solvent to the sodium stannite bleach bath to reduce highlight stain. One volume of tertiary butyl alcohol to about ten volumes of the bleach bath appears to be a satisfactory solvent for this purpose.

Other dyes which, for example, may be bleached in the manner of my invention are: Diphenyl Fast Green BL, Diamine Golden yellow No. 529 Schultz 7th ed. 1931, Brilliant Carmine LS No. 327 Schultz 7th ed. 1931, tetrazotized 4,4'-diaminotriphenylmethane coupled with N-lauroyl H-acid, Diphenyl Brilliant Pink B.

It is to be understood that the disclosure herein is by way of example and that I consider as included in my invention all modifications and equivalents falling within the scope of the appended claims.

What I claim is:

1. The method of forming a colored image in a photographic layer containing uniformly dispersed therein a dye bleachable with a reducing bleach bath under influence of a silver image and a silver image, which comprises rehalogenizing said silver image, converting said rehalogenized image to a silver image, and without intervening treatment, bleaching the dye in the region of the freshly redeveloped silver image with a reducing bleach bath.

2. The method of forming a colored image in a photographic layer containing uniformly dispersed therein a bleachable dye selected from the group consisting of bleachable azo and vat dyes and a silver image, which comprises rehalogenizing said silver image, converting said rehalogenized image to a silver image, and immediately and without intervening treatment, bleaching the dye in the region of the freshly developed silver image with a reducing bleach bath.

3. The method of forming a colored image in a photographic layer containing a bleachable dye selected from the group consisting of bleachable azo and vat dyes uniformly dispersed therein and a silver image, which comprises rehalogenizing said silver image, converting said rehalogenized image to a silver image, and immediately and without intervening treatment, bleaching the dye in the region of the freshly developed silver image with an alkaline reducing bleach bath.

4. The method of forming a colored image in a photographic layer containing a bleachable azo dye uniformly dispersed therein and a silver image, which comprises rehalogenizing said silver image, converting said rehalogenized image to a silver image, and immediately and without intervening treatment, bleaching the dye in the region of the freshly developed silver image with an alkaline reducing bleach bath.

5. The method of forming a colored image in

a photographic layer containing a bleachable azo dye uniformly dispersed therein and a silver image, which comprises rehalogenizing said silver image, converting said rehalogenized image to a silver image, and immediately and without intervening treatment, bleaching the dye in the region of the freshly developed silver image with an alkali stannite bleach bath.

6. The method of forming a colored image in 10 a photographic layer containing a bleachable vat dye uniformly dispersed therein and a silver image, which comprises rehalogenizing said silver image, converting said rehalogenized image to a silver image, and immediately and without intervening treatment, bleaching the dye in the region of the freshly developed silver image with an alkaline reducing bleach bath.

7. The method of forming a colored image in 20 a photographic layer containing a bleachable vat dye uniformly dispersed therein and a silver image, which comprises rehalogenizing said silver image, converting said rehalogenized image to a silver image, and immediately and without intervening treatment, bleaching the dye in the region of the freshly developed silver image with an alkali stannite bleach bath.

8. The method of forming a colored image in 30 a photographic layer containing uniformly dispersed therein a dye bleachable with reducing bleach bath under influence of a silver image, and a silver image, which comprises carrying out a plurality of cycles of rehalogenizing said silver image, converting said rehalogenized image to a silver image, and immediately and without intervening treatment, bleaching the dye in the region of the freshly developed silver image with a reducing bleach bath.

9. The method of forming a colored image in 40 a photographic layer containing uniformly dispersed therein a bleachable dye selected from the group consisting of bleachable azo and vat dyes and a silver image, which comprises carrying out a plurality of cycles of rehalogenizing said silver image, converting said rehalogenized silver image to a silver image, and immediately and without intervening treatment, bleaching the dye in the region of the freshly developed silver image with a reducing bleach bath.

10. The method of forming a colored image in 50 a photographic layer containing a bleachable dye selected from the group consisting of bleachable azo and vat dyes uniformly dispersed therein and a silver image, which comprises carrying out a plurality of cycles of rehalogenizing said silver image, converting said rehalogenized image to a silver image, and immediately and without intervening treatment, bleaching the dye in the region of the freshly developed silver image with an alkaline reducing bleach bath.

11. The method of forming a colored image in 60 a photographic layer containing a bleachable azo dye uniformly dispersed therein and a silver image, which comprises carrying out a plurality of cycles of rehalogenizing said silver image, converting said rehalogenized image to a silver image, and immediately and without intervening treatment, bleaching the dye in the region of the freshly developed silver image with an alkaline reducing bleach bath.

12. The method of forming a colored image in 70 a photographic layer containing a bleachable azo dye uniformly dispersed therein and a silver image, which comprises carrying out a plurality of cycles of rehalogenizing said silver image, converting said rehalogenized image to a silver image,

and immediately and without intervening treatment, bleaching the dye in the region of the freshly developed silver image with an alkali stannite bleach bath.

13. The method of forming a colored image in a photographic layer containing a bleachable azo dye uniformly dispersed therein and a silver image, which comprises rehalogenizing said silver image, converting said rehalogenized image to a silver image, immediately and without interven-

ing treatment, bleaching the dye in the region of the freshly developed silver image with an alkali stannite bleach bath, rehalogenizing said last-mentioned silver image, converting said last-mentioned rehalogenized image to a silver image, and immediately and without intervening treatment, bleaching any dye remaining in the region of said last-mentioned silver image with an alkali stannite bleach bath.

GEORGE EHRENFRIED.